# EUROPEAN PATENT SPECIFICATION

(11) **EP 2 742 978 B1**
(45) Date of publication and mention of the grant of the patent: **12.10.2016**
(21) Application number: 12823385.5
(22) Date of filing: 14.08.2012
(51) Int. Cl.: A62D 1/06

(54) **FIRE-EXTINGUISHING COMPOSITION COMPRISING ORGANIC ACID COMPOUND**
FEUERLÖSCHZUSAMMENSETZUNG MIT EINER ORGANISCHEN SÄUREVERBINDUNG
COMPOSITION D'EXTINCTION D'INCENDIE CONTENANT UN COMPOSÉ D'ACIDE ORGANIQUE

(30) Priority: 16.08.2011 CN 201110235101
(43) Date of publication of application: 18.06.2014
(73) Proprietor: Xi'an Westpeace Fire Technology Co., Ltd, Xi'an, Shaanxi 710065 (CN)
(72) Inventor: YAO, Junna, Xi'an Shaanxi 710065 (CN); LIU, Yi, Xi'an Shaanxi 710065 (CN)
(74) Representative: Jennings, Michael John
(86) International application number: PCT/CN2012/080091
(87) International publication number: WO 2013/023575

(56) References cited:
- EP-A1- 1 797 926
- EP-A2- 0 925 808
- AU-A- 5 208 790
- CN-A- 1 131 573
- CN-A- 101 043 919
- CN-A- 101 376 049
- CN-A- 101 664 587
- CN-A- 102 179 024
- CN-A- 102 179 026
- GB-A- 656 315
- JP-A- 2012 005 730
- US-A- 719 833
- US-A1- 2005 116 193
- US-A1- 2005 242 319

## Description

### Technical field

The disclosure belongs to the technical field of aerosol fire extinguishment, and particularly relating to a fire-extinguishing composition that can be heated to be decomposed to generate a fire-extinguishing substance.

### Background

Since the specific objective of replacing the Halon fire extinguishing agent were proposed to each country by the Canada Montreal Convention in 1987, all countries over the world are dedicated to the study on new fire-extinguishing technologies, therefore, the fire-extinguishing technology with high efficiency in fire-extinguishing and without pollution for environment has become the target for people to strive. Since the fire extinguishing systems such as gas fire extinguishing system, powder fire extinguishing system, water type fire extinguishing system and so on are environmentall-friendly, they are widely used as substitutes of the Halon fire extinguishing agent.they

However, all the fire extinguishing system should be stored under high pressure, not only occupy a large volume, but also have the risk of physical explosion during storage. The document "Security Analysis of Gas Fire extinguishing Systems" (Fire Science and Technology 2002 21 (5)) analyzes the risk that exist in gas fire extinguishing system, and enumerates the accidents caused by using the gas fire extinguishing system kept under pressure.

In recent years, people have been studing Halon substitute fire extinguishing substances, wherein the Next Generation Fire Extinguishing Technology Project Group (NGP) of the Building and Fire Research Centre of the U.S. National Institute of Standards and Technology (NIST) have done a tremendous amount of experimental researches in pursuing a variety of novel fire extinguishing substances, the process includes: heating nitrogen, carbon dioxide and CF₃H, and then heating test substances with these high-temperature gases, the test substances are then decomposed under high temperature and acts on the flame together with the gases; According to the experiments, we find that the products generated by heating and decomposing some test substances can significantly improve the fire-extinguishing effect of the nitrogen, carbon dioxide and CF₃H gas (Halon Options Technical Working Conference, April 2001, Albuquerque, NM, Suppression of cup-burner diffusion flames by super-effective chemical inhibitors and inert compounds; Combustion and Flame 129:221-238(2002) Inhibition of Premixed Methane Flame by Manganese and Tin Compounds, Halon Options Technical Working Conference May 2000, flame inhibition by ferrocene, alone and with CO₂ and CF₃H).

However, the researches of the project group are just based on laboratory theoretical researches, without practical application in fire extinguishers.

Existing aerosol fire extinguishing agents mainly include S type and K- type fire extinguishing agents, by comprehensively analyzing the performance characteristics, the disadvantages are mainly as follows: all the aerosol fire extinguishing agents use fire extinguishing agents to generate an oxidation-reduction reaction, which releases a large number of gases and active particles to achieve the chemical and physical combination fire-extinguishing purpose via the chain scission reaction of the active particles and the coverage smothering of the large number of gases. Aerosol generating agents can release fire-extinguishing substances during combustion reactions while releasing a large amount of heat. In order to effectively lower the temperature of a device and an aerosol, and avoid a secondary fire, a cooling system needs to be installed, which causes a complex and bulky device structure, complex technical process and high cost. Because of the existence of the cooling system, a large number of active particles are inactivated, and the performance of the fire extinguishing is greatly reduced.

Document CN101376049 discloses a hot aerosol fire-extinguishing composition comprising 40%-70% of an oxidizing agent, 20%-50% of a reducing agent, 2%-10% of an adhesive and 2%-20% of a carboxylic acid and/or its salt selected from hydroxybenzoic acid, benzoic acid, palmic acid and o-phthalic acid.

### Summary

In order to solve the above technical problems existing in fire-extinguishing compositions in the prior art, the inventor invents a fire-extinguishing composition comprising an organic acid compound with better fire-extinguishing effect and higher safety performance.

A technical solution applied by the disclosure as follows:
a fire-extinguishing composition comprising an organic acid compound is special in that: the fire-extinguishing composition comprises an organic acid compound; wherein the content of the organic acid compound is 50% by mass or more, and preferably 70% to 90% by mass; the organic acid compound according the disclosure may absorb heat and be decomposed at a high temperature, and release a fire-extinguishing substance, the fire-extinguishing substance may react, by means of free radicals, with one or more of O·, OH·, H·free radicals that are necessary for chemical-looping combustion, thus cutting off the chemical-looping combustion, or may reduce the oxygen partial pressure by physical action to inhibit the flame, or achieve the fire-extinguishing effect by both the physical and chemical inhibition effects. At the same time, the organic acid compound achieves a synergistic effect together with a pyrotechnic agent, thereby further improving the fire-extinguishing performance of the fire-extinguishing agent, and greatly shortening the effective fire-extinguishing time.

To improve the fire-extinguishing performance of the main fire-extinguishing material, i.e. the organic acid compound, a flame retardant may be further added to the above fire-extinguishing composition, i.e. a bromine-based flame retardant, a chlorine-based flame retardant, an organophosphorus-based flame retardant, a phosphorus-halogen based flame retardant, a nitrogen-based and phosphorus-nitrogen flame retardant, or other flame retardants, or any combination thereof, and specifically may be diammonium phosphate, ammonium dihydrogen phosphate, dicyandiamide, melamine, tetrabromobisphenol A, tetrachlorobisphenol A, decabromodiphenyl ether, DOPO, tris(dibromophenyl)phosphate, monomelamine phosphate, guanidine phosphate, guanidine carbonate, ammonium polyphosphate and so on; wherein the content of the flame retardant in the fire-extinguishing composition is smaller than 50% by mass, or may be below 40%, preferably below 30%, and optimally 4% to 25%.

To improve the processability of the main fire-extinguishing material, i.e. the organic acid compound, an additive may be further added to the fire-extinguishing composition of the disclosure, wherein the content of the additive is 0.1 % to 10% by mass, preferably 0.1 % to 5%; the additive may be a water-soluble compound solution or a mixture thereof of a stearate, graphite, and a polymer, or may be also one or more of water glass, phenol resin, shellac and starch, which depends on application conditions.

An auxiliary fire-extinguishing material may be further added to the fire-extinguishing composition of the disclosure in a content that may be controlled at 0% to 30% by mass, preferably 4% to 25%; the auxiliary fire-extinguishing material may be selected from ferrocene or ferrocenyl derivatives, or a mixture of ferrocene and the derivatives thereof, or may be also one or a combination of manganese carbonate, basic copper carbonate, basic magnesium carbonate, ferrous carbonate, potassium citrate, sodium citrate, ammonium citrate, ammonium ferric citrate, potassium oxalate, sodium oxalate, ammonium oxalate, iron oxalate, magnesium oxalate, manganese oxalate and copper oxalate.

The organic acid compound of the disclosure may be capric acid, dodecanoic acid, tetradecanoic acid, hexadecanoic acid, heptadecanoic acid, octadecanoic acid, eicosanoic acid, docosanoic acid, hexacosanoic acid, hentriacontylic acid, dotriacontanoic acid, crotonic acid, oleic acid, heptadecenoic acid, hexadecenoic acid, hexadienic acid, oxalic acid, malonic acid, succinic acid, glutaric acid, pimelic acid, suberic acid, sebacic acid, brassylic acid, hexadecanedioic acid, cis-crotonic acid, trans-crotonic acid, 2-hydroxypropionic acid, 2-hydroxybutanedioic acid, 2,3-dihydroxybutanedioic acid, 2-hydroxy-1,2,3-propanetricarboxylic acid, 3-phenyl-2-propenoic acid, 2-hydroxybenzoic acid, 3,4,5-trihydroxy benzoic acid, benzoic acid or methylguanidoacetic acid.

The fire-extinguishing composition comprising an organic acid compound of the disclosure has the following advantages:
firstly, the fire-extinguishing composition of the disclosure comprises an organic acid compound and is capable of releasing a fire extinguishing substance at the moment of being heated to be decomposed, so as to extinguish a fire using a physical or chemical inhibition effect, or a physical and chemical synergistic inhibition effect of the fire extinguishing substance; in addition, the fire-extinguishing composition of the disclosure also optimizes for the content of the main fire-extinguishing material to exert the best fire-extinguishing effect, so that the fire-extinguishing effect is greatly improved, the fire-extinguishing time is shortened and the fire-extinguishing efficiency of the fire-extinguishing composition is improved.
secondly, a flame retardant, an additive, and other auxiliary fire-extinguishing materials are added to the fire-extinguishing composition of the disclosure, thus further improving the fire-extinguishing performance and processability of the main fire-extinguishing material, i.e. the organic acid compound, making the fire-extinguishing composition stable in performance and easy in long-term storage.
thirdly, the fire-extinguishing composition of the disclosure is more convenient in using with pyrotechnic agent as a heat source.
fourthly, when heated, the fire-extinguishing composition of the disclosure can absorb heat and be decomposed rapidly, thus effectively and rapidly reducing the heat released by combustion of the pyrotechnic agent, greatly reducing the temperature of the nozzle of the fire-extinguishing apparatus and the sprayed substance and achieving higher safety.

### Detailed description of the embodiments

Embodiments of a fire-extinguishing composition comprising an organic acid compound of the disclosure will be described as below in conjunction with experiments:
the fire-extinguishing composition contains an organic acid compound, wherein the content of the organic acid compound is 50% by mass or more, preferably 70% to 90% by mass, and the organic acid compound may be selected from capric acid, dodecanoic acid, tetradecanoic acid, hexadecanoic acid, heptadecanoic acid, octadecanoic acid, eicosanoic acid, docosanoic acid, hexacosanoic acid, hentriacontylic acid, dotriacontanoic acid, crotonic acid, oleic acid, heptadecenoic acid, hexadecenoic acid, hexadienic acid, oxalic acid, malonic acid, succinic acid, glutaric acid, pimelic acid, suberic acid, sebacic acid, brassylic acid, hexadecanedioic acid, cis-crotonic acid, trans-crotonic acid, 2-hydroxypropionic acid, 2-hydroxybutanedioic acid, 2,3-dihydroxybutanedioic acid, 2-hydroxy-1,2,3-propanetricarboxylic acid, 3-phenyl-2-propenoic acid, 2-hydroxybenzoic acid, 3,4,5-trihydroxy benzoic acid, benzoic acid or methylguanidoacetic acid etc., and all these can absorb heat to be decomposed at a high temperature to release a fire-extinguishing substance. The fire-extinguishing substance may react, by means of free radicals, with one or more of O·, OH·, H· free radicals that are necessary for chemical-looping combustion, thus cutting off the chemical-looping combustion, or may reduce the oxygen partial pressure by physical action to inhibit the flame, or achieve the fire-extinguishing effect by both the physical and chemical inhibition effects. At the same time, the organic acid compound achieves a synergistic effect together with a pyrotechnic agent, thereby further improving the fire-extinguishing performance of the fire-extinguishing agent, and greatly shortening the effective fire-extinguishing time.

To improve the fire-extinguishing performance of the main fire-extinguishing material, i.e. the organic acid compound, a flame retardant may be further added to the fire-extinguishing composition, i.e. a bromine-based flame retardant, a chlorine-based flame retardant, an organophosphorus-based flame retardant, a phosphorus-halogen based flame retardant, a nitrogen-based and phosphorus-nitrogen flame retardant, an inorganic flame retardant, or any combination thereof, and specifically may be diammonium phosphate, ammonium dihydrogen phosphate, dicyandiamide, melamine, tetrabromobisphenol A, tetrachlorobisphenol A, decabromodiphenyl ether, DOPO, tris(dibromophenyl)phosphate, monomelamine phosphate, guanidine phosphate, guanidine carbonate, , ammonium polyphosphate and so on, and is not limited thereby, any flame retardant that can be mixed with the organic acid compound to achieve a good fire-extinguishing effect may be applied. wherein the content of the flame retardant in the fire-extinguishing composition is smaller than 50% by mass, or may be below 40%, preferably below 30%, and optimally 4% to 25%, which is adjusted according to specific proportions.

To improve the processability of the main fire-extinguishing material, i.e. the organic acid compound, an additive may be further added to the fire-extinguishing composition of the disclosure, wherein the content of the additive is 0.1 % to 10% by mass, preferably 0.1 % to 5%; the additive may be a water-soluble compound solution or a mixture thereof of a stearate, graphite, and a polymer, or may be also one or more of water glass, phenol resin, shellac and starch, which depends on application conditions, wherein the additive contains an adhesive which belongs to general knowledge in the art. Generally, the content of the additive in the fire-extinguishing composition is controlled below 15% by mass.

An auxiliary fire-extinguishing material may be further added to the fire-extinguishing composition of the disclorure in a content that may be controlled at 0% to 30% by mass, preferably 4% to 25%; the auxiliary fire-extinguishing material may be selected from ferrocene or ferrocenyl derivative, or a mixture of ferrocene and the derivatives thereof, or may be also one or a combination of manganese carbonate, basic copper carbonate, basic magnesium carbonate, ferrous carbonate, potassium citrate, sodium citrate, ammonium citrate, ammonium ferric citrate, potassium oxalate, sodium oxalate, ammonium oxalate, iron oxalate, magnesium oxalate, manganese oxalate and copper oxalate.

65g of a prepared tablet fire-extinguishing composition is respectively added to a fire-extinguishing apparatuses charged with a 50g K-type hot aerosol generating agent to carry out fire-extinguishing tests according to Term 6.3.2 of GA86-2009 respectively at a fire-extinguishing level of 8B. The test results are as shown in Table 1, and 50g of a commercially available K-type hot aerosol generating agent is applied in a comparison example.

**Table 1 Comparison of various composition components and comparison of test results**

| Components | Component content of embodiments (mass percent) | | | | | | | | | | | | Comparison example |
|---|---|---|---|---|---|---|---|---|---|---|---|---|---|
| | 1 | 2 | 3 | 4 | 5 | 6 | 7 | 8 | 9 | 10 | 11 | 12 | 50g of commercially available K-type hot aerosol generating agent |
| capric acid | 70 | | | | | | | | | | | | |
| hexadienic acid | | 75 | | | | | | | | | | | |
| oxalic acid | | | 79.8 | | | | | | | | | | |
| malonic acid | | | | 80 | | | | | | | | | |
| succinic acid | | | | | 80 | | | | | | | | |
| 2-hydroxybutanedioic acid | | | | | | 75 | | | | | | | |
| 2,3-dihydroxybutanedioic acid | | | | | | | 70 | | | | | | |
| 2-hydroxy-1,2, 3-propanetricarboxylic acid | | | | | | | | 75 | | | | | |
| 3-phenyl-2-propenoic acid | | | | | | | | | 80 | | | | |
| 2-hydroxybenzoic acid | | | | | | | | | | 80 | | | |
| 3,4,5-trihydroxy benzoic acid | | | | | | | | | | | 85 | | |
| N-methylguanidinoacetic acid | | | | | | | | | | | | 85 | |
| ammonium oxalate | 19 | | | | | | | | 5 | | | | |
| melamine | | | | 4 | | 9 | 25 | 9.5 | | 19 | | 1.5 | |
| manganese carbonate | | 14 | | | | 10 | | | 5 | | 13 | | |
| potassium citrate | | | | | | | | 15 | | | | 12 | |
| sodium citrate | | | | 15 | | | | | 9 | | | | |
| water glass | | | | 1 | | | | | 1 | | 1 | | |
| magnesium stearate | | | | | 5 | 5 | | | | 0.2 | | 0.5 | |
| zinc stearate | | | | | 5 | | | | | | 1 | | |
| hydroxypropyl | | 1 | 0.2 | | | | 5 | 0.5 | | 0.8 | | | |
| methylcellulose | | | | | | | | | | | | | |
| polyvinyl alcohol | 0.8 | | | | 1 | 1 | | | | | | 1 | |
| ferrocene | 9.2 | 9 | 20 | | 9 | | | | | | | | |
| hydroxyethyl cellulose | 1 | 1 | | | | | | | | | | | |
| nozzle temperature of generator (°C) | 92 | 97 | 100 | 120 | 98 | 142 | 103 | 76 | 89 | 85 | 69 | 106 | 469 |
| fire-extinguishing result | x | x | x | x | x | x | x | x | x | x | x | x | y |
| fire-extinguishing time (s) | 8.1 | 6.4 | 5.6 | 3.7 | 6.1 | 4.8 | 7.3 | 4.6 | 6.7 | 5.8 | 6.4 | 7:5 | |

| | | | | | | | | | | | | | |
|---|---|---|---|---|---|---|---|---|---|---|---|---|---|
| X = extinguished Y = not extinguished | | | | | | | | | | | | | |

It can be clearly seen from Table 1 that the fire-extinguishing efficiency of compositions using the organic acids in the first to the twelfth embodiments of the disclosure as main fire-extinguishing materials are far better than that in the comparison example, and the fire-extinguishing time is shorter and the generator nozzle temperature is lower than those in the comparison example.

## Claims

1. Afire-extinguishing composition comprising an organic acid compound, wherein the fire-extinguishing composition comprises an organic acid compound; the content of the organic acid compound is 50% by mass or more;
A pyrotechnic agent is adopted as a heat source and a power source of the fire extinguishing composition; and the purpose of fire extinguishing is achieved by: igniting the pyrotechnic agent, and the fire extinguishing composition performing decomposition reaction and generating a large quantity of fire extinguishing substance under high temperature produced by burning of pyrotechnic agent, and the fire extinguishing substance sprayed out together with the pyrotechnic agent from a nozzle.

2. The fire-extinguishing composition comprising an organic acid compound according to claim 1, wherein the composition further comprises an auxiliary fire-extinguishing material; the auxiliary fire-extinguishing material is one or more of a citrate, an oxalate, a carbonate, ferrocene or ferrocenyl derivative, and the content thereof is more than 0, and less than or equal to 30% by mass.

3. The fire-extinguishing composition comprising an organic acid compound according to claim 1, wherein the composition further comprises a flame retardant; the content of the flame retardant is more than 0, and less than or equal to 50% by mass.

4. The fire-extinguishing composition comprising an organic acid compound according to any one of claims 1 to 3, wherein the composition further comprises an additive; the content of the additive is 0.1 % to 10% by mass.

5. The fire-extinguishing composition comprising an organic acid compound according to claim 4, wherein the additive is a water-soluble compound solution or a mixture of a stearate, graphite, and a polymer, or is one or more of water glass, phenol resin, shellac and starch.

6. The fire-extinguishing composition comprising an organic acid compound according to claim 4, wherein the organic acid compound is capric acid, dodecanoic acid, tetradecanoic acid, hexadecanoic acid, heptadecanoic acid, octadecanoic acid, eicosanoic acid, docosanoic acid, hexacosanoic acid, hentriacontylic acid, dotriacontanoic acid, crotonic acid, oleic acid, heptadecenoic acid, hexadecenoic acid, hexadienic acid, oxalic acid, malonic acid, succinic acid, glutaric acid, pimelic acid, suberic acid, sebacic acid, brassylic acid, hexadecanedioic acid, cis-crotonic acid, trans-crotonic acid, 2-hydroxypropionic acid, 2-hydroxybutanedioic acid, 2,3-dihydroxybutanedioic acid, 2-hydroxy-1,2,3-propanetricarboxylic acid, 3-phenyl-2-propenoic acid, 2-hydroxybenzoic acid, 3,4,5-trihydroxy benzoic acid, benzoic acid or methylguanidoacetic acid.

7. The fire-extinguishing composition comprising an organic acid compound according to claim 6, wherein the content of the organic acid compound is preferably 70% to 90% by mass.

8. The fire-extinguishing composition comprising an organic acid compound according to claim 3, wherein the flame retardant is a bromine-based flame retardant, a chlorine-based flame retardant, an organophosphorus-based flame retardant, a phosphorus-halogen based flame retardant, a nitrogen-based and phosphorus-nitrogen flame retardant, other flame retardants, or any combination thereof.

9. The fire-extinguishing composition comprising an organic acid compound according to claim 8, wherein the content of the flame retardant is more than 0 and less than 30% by mass.

10. The fire-extinguishing composition comprising an organic acid compound according to claim 1, wherein the fire-extinguishing composition further comprises:
an auxiliary fire-extinguishing material 4% to 25% by mass;
| | |
|---|---|
| a flame retardant | 4% to 25% by mass; |
| an additive | 0.1 % to 5% by mass. |

## Patentansprüche

1. Eine organische Säureverbindung umfassende Feuerlöschzusammensetzung, wobei die Feuerlöschzusammensetzung eine organische Säureverbindung umfasst; wobei der Gehalt der organischen Säureverbindung 50 Massen-% oder mehr beträgt;
wobei ein pyrotechnisches Mittel als eine Wärmequelle und eine Energiequelle der Feuerlöschzusammensetzung eingesetzt wird und die Absicht des Feuerlöschens durch Folgendes erzielt wird: Zünden des pyrotechnischen Mittels und Durchführen einer Zersetzungsreaktion und Erzeugen einer großen Menge an Feuerlöschsubstanz unter hoher Temperatur durch die Feuerlöschzusammensetzung, die durch Abbrennen des pyrotechnischen Mittels hervorgerufen wird, und wobei die Feuerlöschsubstanz zusammen mit dem pyrotechnischen Mittel aus einer Düse gesprüht wird.

2. Eine organische Säureverbindung umfassende Feuerlöschzusammensetzung nach Anspruch 1, wobei die Zusammensetzung weiterhin ein Hilfsfeuerlöschmaterial umfasst; das Hilfsfeuerlöschmaterial eines oder mehrere von einem Citrat, einem Oxalat, einem Carbonat, einem Ferrocen oder Ferrocenylderivat ist und der Gehalt davon größer als 0 und kleiner gleich 30 Massen-% ist.

3. Eine organische Säureverbindung umfassende Feuerlöschzusammensetzung nach Anspruch 1, wobei die Zusammensetzung weiterhin ein flammenhemmendes Mittel umfasst; wobei der Gehalt des flammhemmenden Mittels größer als 0 und kleiner gleich 50 Massen-% ist.

4. Eine organische Säureverbindung umfassende Feuerlöschzusammensetzung nach einem der Ansprüche 1 bis 3, wobei die Zusammensetzung weiterhin ein Additiv umfasst;
wobei der Gehalt des Additivs 0,1 Massen-% bis 10 Massen-% beträgt.

5. Eine organische Säureverbindung umfassende Feuerlöschzusammensetzung nach Anspruch 4, wobei das Additiv eine Lösung einer wasserlöslichen Verbindung oder ein Gemisch von einem Stearat, Graphit und einem Polymer ist oder eines oder mehrere von einem Wasserglas, Phenolharz, Schellack und Stärke ist.

6. Eine organische Säureverbindung umfassende Feuerlöschzusammensetzung nach Anspruch 4, wobei die organische Säureverbindung Caprinsäure, Dodecansäure, Tetradecansäure, Hexadecansäure, Heptadecansäure, Octadecansäure, Eicosansäure, Docosansäure, Hexacosansäure, Hentriacontansäure, Dotriacontansäure, Crotonsäure, Ölsäure, Heptadecensäure, Hexadecensäure, Hexadiensäure, Oxalsäure, Malonsäure, Bernsteinsäure, Glutarsäure, Pimelinsäure, Korksäure, Sebacinsäure, Brassylsäure, Hexadecandisäure, cis-Crotonsäure, trans-Crotonsäure, 2-Hydroxypropionsäure, 2-Hydroxybutandisäure, 2,3-Dihydroxybutandisäure, 2-Hydroxy-1,2,3-propantricarbonsäure, 3-Phenyl-2-propensäure, 2-Hydroxybenzoesäure, 3,4,5-Trihydroxybenzoesäure, Benzoesäure oder Methylguanidoessigsäure ist.

7. Eine organische Säureverbindung umfassende Feuerlöschzusammensetzung nach Anspruch 6, wobei der Gehalt der organischen Säureverbindung vorzugsweise 70 Massen-% bis 90 Massen-% beträgt.

8. Eine organische Säureverbindung umfassende Feuerlöschzusammensetzung nach Anspruch 3, wobei es sich bei dem flammhemmenden Mittel um ein flammhemmendes Mittel auf Brombasis, ein flammhemmendes Mittel auf Chlorbasis, ein flammhemmendes Mittel auf Organophosphorbasis, ein flammhemmendes Mittel auf Phosphor-Halogen-Basis, ein flammhemmendes Phosphor-Stickstoff-Mittel auf Stickstoffbasis, andere flammhemmende Mittel oder eine beliebige Kombination davon handelt.

9. Eine organische Säureverbindung umfassende Feuerlöschzusammensetzung nach Anspruch 8, wobei der Gehalt des flammhemmenden Mittels größer als 0 und kleiner als 30 Massen-% ist.

10. Eine organische Säureverbindung umfassende Feuerlöschzusammensetzung nach Anspruch 1, wobei die Feuerlöschzusammensetzung weiterhin Folgendes umfasst:
ein Hilfsfeuerlöschmaterial zu 4 Massen-% bis 25 Massen-%;
ein flammhemmendes Mittel zu 4 Massen-% bis 25 Massen-%;
ein Additiv zu 0,1 Massen-% bis 5 Massen-%.

## Revendications

1. Composition d'extinction d'incendie comprenant un composé acide organique, la composition d'extinction d'incendie comprenant un composé acide organique ; la teneur du composé acide organique étant supérieure ou égale à 50 % en masse ;
un agent pyrotechnique étant choisi en tant que source de chaleur et source d'énergie de la composition d'extinction d'incendie ; et la finalité d'extinction d'incendie étant réalisée par : inflammation de l'agent pyrotechnique et le fait que la composition d'extinction d'incendie subit une réaction de décomposition et produit une grande quantité de substance d'extinction d'incendie sous une température élevée produite par la combustion d'agent pyrotechnique et la pulvérisation de la substance d'extinction d'incendie vers l'extérieur conjointement avec l'agent pyrotechnique à partir d'une lance.

2. Composition d'extinction d'incendie comprenant un composé acide organique selon la revendication 1, la composition comprenant en outre une matière d'extinction d'incendie auxiliaire ; la matière d'extinction d'incendie auxiliaire étant une ou plusieurs matières parmi un citrate, un oxalate, un carbonate, le ferrocène ou un dérivé de ferrocényle et la teneur de celle-ci étant supérieure à 0 et inférieure ou égale à 30 % en masse.

3. Composition d'extinction d'incendie comprenant un composé acide organique selon la revendication 1, la composition comprenant en outre un agent ignifugeant ; la teneur de l'agent ignifugeant étant supérieure à 0 et inférieure ou égale à 50 % en masse.

4. Composition d'extinction d'incendie comprenant un composé acide organique selon l'une quelconque des revendications 1 à 3, la composition comprenant en outre un additif ; la teneur de l'additif étant de 0,1 % à 10 % en masse.

5. Composition d'extinction d'incendie comprenant un composé acide organique selon la revendication 4, dans laquelle l'additif est une solution de composé hydrosoluble ou un mélange d'un stéarate, de graphite et d'un polymère ou est un ou plusieurs additifs parmi du verre soluble, de la résine phénolique, de la gomme laque et de l'amidon.

6. Composition d'extinction d'incendie comprenant un composé acide organique selon la revendication 4, dans laquelle le composé acide organique est l'acide caprique, l'acide dodécanoïque, l'acide tétradécanoïque, l'acide hexadécanoïque, l'acide heptadécanoïque, l'acide octadécanoïque, l'acide éicosanoïque, l'acide docosanoïque, l'acide hexacosanoïque, l'acide hentriacontylique, l'acide dotriacontanoïque, l'acide crotonique, l'acide oléique, l'acide heptadécénoïque, l'acide hexadécénoïque, l'acide hexadiénoïque, l'acide oxalique, l'acide malonique, l'acide succinique, l'acide glutarique, l'acide pimélique, l'acide subérique, l'acide sébacique, l'acide brassylique, l'acide hexadécanedioïque, l'acide cis-crotonique, l'acide *trans-*crotonique, l'acide 2-hydroxypropionique, l'acide 2-hydroxybutanedioïque, l'acide 2,3-dihydroxybutanedioïque, l'acide 2-hydroxy-1,2,3-propanetricarboxylique, l'acide 3-phényl-2-propénoïque, l'acide 2-hydroxybenzoïque, l'acide 3,4,5-trihydroxybenzoïque, l'acide benzoïque ou l'acide méthylguanidoacétique.

7. Composition d'extinction d'incendie comprenant un composé acide organique selon la revendication 6, dans laquelle la teneur du composé acide organique est de préférence de 70 % à 90 % en masse.

8. Composition d'extinction d'incendie comprenant un composé acide organique selon la revendication 3, dans laquelle l'agent ignifugeant est un agent ignifugeant à base de brome, un agent ignifugeant à base de chlore, un agent ignifugeant à base d'organophosphoré, un agent ignifugeant à base de phosphore-halogène, un agent ignifugeant de phosphore-azote et à base d'azote, d'autres agents ignifugeants ou une quelconque association de ceux-ci.

9. Composition d'extinction d'incendie comprenant un composé acide organique selon la revendication 8, dans laquelle la teneur de l'agent ignifugeant est supérieure à 0 et inférieure à 30 % en masse.

10. Composition d'extinction d'incendie comprenant un composé acide organique selon la revendication 1, la composition d'extinction d'incendie comprenant en outre :
4 % à 25 % en masse d'une matière d'extinction d'incendie auxiliaire ;
4 % à 25 % en masse d'un agent ignifugeant ;
0,1 % à 5 % en masse d'un additif.
